

Dec. 14, 1937.

C. L. HARDWICK

2,102,530

METHOD OF MAKING BURNERS

Filed May 29, 1936

2 Sheets-Sheet 1

Fig. 1.



Fig. 2.



INVENTOR  
*Christopher L. Hardwick.*

BY *Fisher, Moore & Moore*  
ATTORNEYS

Dec. 14, 1937.

C. L. HARDWICK

2,102,530

METHOD OF MAKING BURNERS

Filed May 29, 1936

2 Sheets-Sheet 2

Fig. 3



Fig. 4



Fig. 5.



INVENTOR

Christopher L. Hardwick.

BY Fisher, Moser & Moore

ATTORNEYS

## UNITED STATES PATENT OFFICE

2,102,530

## METHOD OF MAKING BURNERS

Christopher L. Hardwick, Cleveland, Tenn.

Application May 29, 1936, Serial No. 82,604

3 Claims. (Cl. 22—200)

This invention relates to a method of casting one piece burners having a continuous relatively narrow annular horizontally arranged combustion opening or slot.

According to present practice such burners are cast with solid walls or sides, and the combustion slot or opening is then formed with a cutting tool, such as disclosed in my prior Patent No. 2,022,857, granted December 3, 1935. This machine method has been practiced due to the fact that it has been found impossible to form the combustion slot by ordinary casting methods. The gas slot is relatively narrow, that is, approximately  $\frac{1}{16}$  of an inch in width, thus making it impracticable to employ a baked sand core having a sufficiently thin projection or flange to form a slot of such narrow width, due to the fact that the flange or projection would break down when the molten metal is poured.

An object of the present invention is to overcome the foregoing objections by providing a method whereby the combustion slot can be formed simultaneously with the casting operation.

Other and more specific objects and advantages of the invention will be apparent from the following description considered with the accompanying drawings, in which:

Figure 1 is a side elevation of a burner casting having an annular combustion slot formed therein according to my invention;

Figure 2 is a sectional view through a mold showing the novel core and the slotted casting therein, the transverse core being omitted;

Figure 3 is a plan view of the lower or drag portion of the mold, the casting and cores being shown in section, the section being taken on the mold junction line 3—3 of Figure 2;

Figure 4 is a perspective view of the main core with the slot forming auxiliary core member in place thereon; and

Figure 5 is a perspective view of the slot-forming or auxiliary transverse core member.

Referring more particularly to the drawings B denotes a gas burner made according to my improved method, and adapted for use with gas stoves, hot air furnaces, steam and hot water boilers. The burner B consists of a hollow integral casting 1, one end of which forms an elongated mixing tube 2 and the other end of which forms the body or burner part 3. Gas is fed through the tube 2 to a ring-shaped distributing and mixing chamber 4, and from there is discharged through a horizontally disposed annular slot 5, where combustion occurs. A through

opening 6, surrounded by the wall of chamber 4, insures an adequate supply of secondary air to the flame.

The slot 5 is formed during and simultaneously with the casting of the burner. Thus a baked sand core 7 of substantially the same size and contour as casting 1, is suitably positioned in a two part flask or mold 8 for the conventional pouring operation. In the present embodiment the flask or mold 8 comprises a lower half or drag portion 9, and an upper half or cope portion 10, as illustrated in Figures 2 and 3. A second and intersecting baked sand core 11, shown in Figure 3 is also inserted in the flask for an obvious purpose. It will be noted that the body or burner portion 12 of the core 7, carries a ring-shaped auxiliary core member 13, which is designed to keep the molten metal from contacting with that area of the sand core immediately back of or adjacent to the space comprising the slot 5 in the completed casing 1, thus keeping this space open during the casting operation. The ring-shaped auxiliary core member 13, which is made of any suitable non-combustible material, which is not sufficiently fragile to become broken or distorted by flowing metal, is preferably slipped over the mouth of the sand core 7 after the core has been baked, as best illustrated in Figures 3 and 4 of the drawings. Rings 13 made of asbestos paper have proven very satisfactory because rings of this material, are not only highly resistant to heat, and sufficiently strong to withstand the strains and stresses incident to the casting operation, but can be readily removed after the casting 1 has been made. The core member 13, must project from the baked sand core 7, and in reality constitutes a relatively thin flange. Such a thin flange formed of baked sand has been found to be utterly impracticable due to the fragile nature of baked sand.

It will be understood that when the molten metal is poured into the gates or pouring openings 14 and 15 of mold 8, the metal will flow about the cores 7 and 11 to form a casting 1, having the slot 5 formed therein. The ring-shaped non-combustible auxiliary core member 13 remains unbroken and undistorted by the molten metal and consequently the slot 5 will be accurately formed. After the casting has cooled and the baked cores 7 and 11 broken down and the sand poured out of the casting, in a manner well known to workers in the art, the ring-shaped slot forming member 13 is removed. Any suitable hand tool may be employed for removing the ring 13 from the casting. In addition to functioning

as an auxiliary core member the ring 13 serves to anchor the core in the sand of the flask or mold.

Having thus described my invention, what I claim is:

- 5 1. The method of casting round burners having a hollow body and a relatively thin annular combustion slot comprising the steps of forming a baked sand core having the outline of said body, placing a ring-shaped auxiliary core member of 10 strong non-combustible material on said baked sand core and inserting said baked sand core and said auxiliary core in a previously prepared mold whereby, when metal is cast in said mold, the space occupied by said auxiliary core will constitute said slot.
- 15 2. The method of casting round burners having a hollow body and a relatively thin annular combustion slot intersecting one wall, comprising the steps of forming a baked sand core having the 20 outline of said body, placing a flat washer shaped auxiliary core member of strong non-combustible material on one edge of said sand core and extending beyond the side wall thereof and placing the same in the mold with the greater portion of the flat face of the auxiliary core spaced from the sand of the mold and the edges em-

bedded in the sand for supporting the core whereby when metal is cast in said mold, the space occupied by the thickness of the flat washer shaped core will constitute a slot in one wall of the body.

- 5 3. The method of casting round burners having a hollow body portion and a relatively thin annular combustion slot intersecting one wall, comprising the steps of forming a baked sand core having the outline of said body, and placing a 10 second sand core transversely through an opening in said first core and spaced therefrom, placing a flat washer shaped auxiliary core member of strong non-combustible material on one edge of said first sand core and spaced from the second transverse sand core and placing the same in the mold with the greater portion of the flat face of the auxiliary core spaced from the sand of the mold and a small portion of the same embedded in the sand for supporting the core whereby when the metal is cast in said mold the space occupied by the thickness of the flat washer shaped core will constitute a slot in one wall of the body.

CHRISTOPHER L. HARDWICK.

25